

Nov. 29, 1955

H. R. STROBEL

2,725,353

ELECTROPOOLISHING METALLIC ARTICLES

Filed July 21, 1950

5 Sheets-Sheet 1



FIG. 1



FIG. 2

INVENTOR  
H. R. STROBEL  
BY *John H. Strobel*  
ATTORNEY

Nov. 29, 1955

H. R. STROBEL

2,725,353

ELECTROPOLISHING METALLIC ARTICLES

Filed July 21, 1950

5 Sheets-Sheet 2



FIG. 3

INVENTOR  
H. R. STROBEL  
BY *John M. Nany*  
ATTORNEY

Nov. 29, 1955

H. R. STROBEL

2,725,353

ELECTROPOLISHING METALLIC ARTICLES

Filed July 21, 1950

5 Sheets-Sheet 3



FIG. 4

INVENTOR  
H. R. STROBEL  
BY *John M. Mang*  
ATTORNEY

Nov. 29, 1955

H. R. STROBEL

2,725,353

ELECTROPOHLISHING METALLIC ARTICLES

Filed July 21, 1950

5 Sheets-Sheet 4



F/G. 5

ALKALINE  
NEUTRALIZING  
22

RINSING  
120



F/G. 6

INVENTOR  
H. R. STROBEL  
BY *John M. Lang*  
ATTORNEY

Nov. 29, 1955

H. R. STROBEL

2,725,353

ELECTROPOLISHING METALLIC ARTICLES

Filed July 21, 1950

5 Sheets-Sheet 5



INVENTOR  
H. R. STROBEL  
BY *Lefty Lang*  
ATTORNEY

# United States Patent Office

2,725,353

Patented Nov. 29, 1955

1

2,725,353

## ELECTROPOLISHING METALLIC ARTICLES

Herman R. Strobel, Fullerton, Md., assignor to Western Electric Company, Incorporated, New York, N. Y., a corporation of New York

Application July 21, 1950, Serial No. 175,124

6 Claims. (Cl. 204—32)

This invention relates to electropolishing metallic articles, and more particularly to electropolishing metallic filaments, such as tapes, wires and the like.

Certain types of communication systems employ coaxial cable units of the type in which an outer tubular conductor made from a metallic tape is supported concentrically on a central, wire-like, conductor by spaced insulating discs, or the like. In the manufacture of such a coaxial unit, it is important that the inner surface of the tape and the surface of the central conductor used in making it be free of ridges, splinters, bumps, flakes and other projections in order for the electrical characteristics of the unit to be uniform throughout the length of the unit. In the past, this result has been difficult to achieve. Other industries also require metallic articles having smooth, polished surfaces.

An object of the invention is to provide new and improved methods of electropolishing metallic articles.

A further object of the invention is to provide new and improved methods of electropolishing metallic filaments, such as tapes, wires and the like.

Another object of the invention is to provide new and improved methods of removing splinters, metallic flakes, ridges and other projections from the copper wires and tapes used in making coaxial cable units.

A method illustrating certain features of the invention may include immersing a copper article to be polished in an aqueous electrolyte including copper nitrate and sulphuric acid, and making the article an anode, whereby projections on the surface of the article are dissolved and the surface of the article is passivated.

A complete understanding of the invention may be obtained from the following detailed description of methods forming specific embodiments thereof, when read in conjunction with the appended drawings, in which:

Fig. 1 is a front elevation of a portion of an apparatus for effecting one method embodying the invention;

Fig. 2 is a corresponding view of another portion of the apparatus continued from the right hand end of Fig. 1;

Fig. 3 is an enlarged, partially sectional view of a portion of the apparatus shown in Fig. 1;

Fig. 4 is an enlarged, vertical section taken along line 4—4 of Fig. 3;

Fig. 5 is a front elevation of a portion of another apparatus for effecting a method forming one embodiment of the invention;

Fig. 6 is a corresponding view of another portion of the apparatus continued from the right hand end of Fig. 5;

Fig. 7 is an enlarged, top plan view of a portion of the apparatus shown in Fig. 5;

Fig. 8 is a vertical section taken along line 8—8 of Fig. 7, and

Fig. 9 is a view of a portion of one type of tape which may be treated by methods and baths embodying the invention.

Referring now in detail to the drawings, a capstan 8 (Fig. 1) advances a filamentary copper conductor 10 of substantial length to be polished continuously through a

2

cleaning bath 12, rinsing bath 14, a cathode device 16 immersed in an electropolishing bath 18, a rinsing bath 20, an alkaline neutralizing bath 22 and a rinsing bath 24. The conductor 10 is advanced by the capstan 8 from a suitable supply reel (not shown) to a takeup reel 25. A rotary contact sheave 34 contacts the conductor 10 at a point in advance of the entrance thereof into the electropolishing bath 18, and the sheave 34 is connected to the positive side of a source of D. C. potential (not shown), the negative side of which is connected to the cathode device 16. The bath 12 is an alkaline bath, and removes grease and foreign substances from the surface of the conductor as it is advanced therethrough. The rinsing bath 14 is water, which rinses any alkali on the conductor therefrom.

The cathode device 16 includes hollow, plastic cylinders 39 and 40 (Figs. 3 and 4), around which smooth, endless, stainless steel or copper sheet cathodes 42—42 are guided and continuously advanced. The cylinders 20 are composed of insulating material, such as, for example, the phenol-formaldehyde condensation product "Bakelite," and are provided with a series of perforations 41—41 and extending therethrough. Cathode rolls 44—44 advance and contact the sheet cathodes 42—42, and 25 guide rolls 46—46 guide the cathodes around the cylinders. The cathodes 42—42 are advanced continuously and scrapers 48—48 scrape copper deposited on the cathodes from the smooth surfaces thereof.

The area of the perforations in the cylinder 39 with 30 respect to the surface area of the portion of the conductor 10 coextensive therewith is sufficiently small to limit the flow of current between the conductor and the sheet cathode on the cylinder 39 to an amount less than that at which passivation of the surface of the conductor 35 occurs. The area of the perforations per unit of length of the cylinders 39 and 40 gradually increases from the entrance of the cylinder 39 to a point on the cylinder 40 about two thirds of the combined length of the cylinders 39 and 40 from the entrance end of the cylinder 39 to an extent that from the point about two thirds of the distance from the exit end of the cylinder 40 to the exit end of the cylinder 40 sufficient current flows from the conductor to the sheet cathode to passivate rapidly the surface of the conductor and to electropolish that surface. The latter portion of the bath may be termed the 45 passivating portion thereof and the preceding portion may be termed the projection dissolving portion.

The composition of the electropolishing bath 18 should be from about 18% to about 30% by weight copper nitrate, from about 6% to about 2% by weight sulphuric acid, and the balance water. The sulphuric acid increases the conductivity of the electropolishing bath, but the concentration thereof is sufficiently low to prevent precipitating copper sulphate out of the solution, and the concentration of the sulphuric acid within the above-listed range is inverse with respect to the copper nitrate in the solution. The high concentration of copper nitrate supplies the necessary copper ions to the electrolytic solution, and the nitrate radical serves to minimize etching. The addition to the bath of a small amount of chromic acid in amounts up to 2% by weight of the total electrolyte tends to minimize pitting of the article being electropolished. The presence of small amounts of one or more water soluble wetting agents, such as, for example, a sodium salt of an alkyl naphthalene sulphonate acid or an ester 60 of a sulphonated dicarboxylic acid commonly sold under the trade name "Aerosol" also reduces pitting action. Another strong, stable acid, such as, for example, fluoroboric acid, fluosilicic acid, phosphoric acid or a sulfonic acid, may be used in place of the sulphuric acid in an amount which would give the electrolyte substantially the same conductivity as the abovementioned electrolyte.

The temperature of the bath should not be greater than around 110° F. to promote rapid passivation of the surface of the conductor 10, and should not be below about 65° F. to prevent precipitation of copper sulphate from the bath. The optimum temperature range is from about 75° F. to about 90° F. The bath is cooled to a temperature within this range by a suitable cooling unit (not shown).

*Operation of embodiment shown in Figs. 1 to 4*

The conductor 10 is advanced continuously through the apparatus, and the cleaning bath 12 cleans grease and foreign matter from the surface of the conductor. The water rinsing bath 14 rinses any alkali on the conductor 10 therefrom, and the conductor 10 is advanced therefrom through the electropolishing bath 18 and the cathode device 16 immersed in the bath 18.

The perforations 41—41 in the cylinder 39 expose only a sufficient area of the sheet cathode 42 therearound to cause projections on the surface of the conductor to dissolve without passivating the surface of the conductor, the current density on the conductor within the cylinder 39 being below 3,000 amperes per square foot. The exposed area of the sheet cathodes 42—42 becomes progressively and uniformly greater from the entrance end of the cylinder 39 to a point on the cylinder 40 about one third of its length from the entrance end thereof, and the current density on the conductor from that point to the exit end of the cylinder 40, averages at least 3,000 amperes per square foot.

After the larger projections on the surface of the conductor have been dissolved into the electrolyte in the projection-dissolving portion of the bath, the increased current density electropolishes and passivates the surface of the conductor. As the electropolishing proceeds under the high current density, the portion of the solution immediately surrounding the conductor is broken-down sufficiently to make oxygen abundantly available at the surface of the conductor, and copper oxides build up on the conductor sufficiently to passivate the surface of the conductor after the surface has received a high polish. The passivating oxide layer substantially prevents further erosion. The electrolyte is recirculated slowly to prevent agitation, and the conductor 10 is advanced through the bath 16 sufficiently slowly to insure substantially no agitation of the electrolyte around the surface of the conductor, which facilitates passivation.

In one specific example, the electropolishing bath 18 consisted of 19% copper nitrate, 4.5% sulphuric acid and the balance water, and was maintained at a temperature of from about 80° F. to about 85° F. Sulphuric acid was added to the bath in dilute solution at intervals to the extent necessary to maintain the correct concentration thereof in the bath. In that example, the width of each of the cathodes 42—42 was about eight inches, and the time of the passage of the conductor through the electrode device 16 was between five and ten seconds. The diameter of the conductor was 0.1009 inch, the spacing between the cathodes 42—42 and the conductor was  $\frac{1}{6}$  inch and the voltage between the conductor and the cathodes was 16 volts.

The ratio of the exposed area of the sheet cathodes to the surface area of the portion of the conductor coextensive therewith varied gradually from about 2 to 3 at the entrance end of the cylinder 39, to about 4 to 1 at the exit end of the projection-dissolving portion of the bath, and remained at a 4 to 1 ratio throughout the passivating portion of the bath. In this example, there was substantially no agitation of the electrolyte around the conductor, and passivation proceeded rapidly. The average current density on the portion of the conductor in the bath 18 was 2,400 amperes per square foot.

The conductor 10 is advanced from the electropolishing bath 18 into and through the rinsing bath 20 and the alkaline neutralizing bath 22, which removes the sur-

face layer of copper oxides to leave a bright, polished surface. The bath 22 may be a water solution of sodium hydroxide, sodium or potassium cyanide, or other suitable alkaline material. After leaving the neutralizing bath 22, the conductor is advanced through the water rinsing bath 24. The conductor then is dried and taken up on suitable reels. The conductor has a lustrous, straw color as it enters the bath 22, and has a smooth, golden colored surface as it leaves that bath.

*Embodiment shown in Figs. 5 to 8*

This apparatus serves to electropolish one face of a copper tape 110 having serrated edges 111—111 (Fig. 9). The tape 110 is advanced continuously by rolls 108—108 through a suitable alkaline cleaning bath 112, a water rinsing bath 114, an electropolishing bath 118 having an electrolyte therein of the same composition as that of the electrolyte in the bath 18, a water rinsing bath 120, an alkaline neutralizing bath 122 and a water rinsing bath 124. The tape 110 is drawn from a supply stand (not shown) and is wound on a suitable takeup device 125.

A rotary contact sheave 134 contacts the tape 110 at a point prior to the entrance of the tape into the bath 118, and is connected to the positive side of a source of D. C. potential (not shown), the negative side of which is connected to a rotary contact sheave 140 (Fig. 7). Feed rolls 142—142 advances a cathode tape 144 through the bath 118 in the same general direction as that in which the tape 110 is advanced therethrough, and guide rolls 145—145 guide the tape 144 in a direction converging toward the tape 110 from the entrance end of the electropolishing bath 118 to the exit end thereof. The cathode tape 144 engages the contact sheave 140, and thereby acquires a negative potential.

As the tape 110 passes through the bath 118, the voltage between the tape 110 and the cathode tape 144, the spacing between the two tapes, and the conductivity of the bath are such that any projections on the surface of the tape 110 are first dissolved therefrom by electrolytic action under an anode current density that is high but below 3,000 amperes per square foot. The anode current density is increased as the tape 110 approaches the exit end of the cell to over 3,000 amperes per square foot to form a layer of copper oxides on the face of the tape 110 nearer the cathode tape 144, and to polish and passivate that face by the time the tape 110 leaves the bath 118.

The bath 118 is contained in a tank 146 supported by a frame 147. A pair of spaced apertures 148—148 are provided at the entrance end of the tank 146 for the passage therethrough of the tapes 110 and 144. The distance between these tapes gradually decreases as they approach the exit end of the tank and emerge through a single aperture 149. A mask 150 composed of a non-conductive material, such as wood or plastic, extends along the bath 118, and covers the back of the tape 110 and the edges 111—111 thereof to prevent dissolving away the serrated edge portions thereof. The mask 150 includes a back 152 having a groove 154 therein, and this mask is supported at opposite ends of the tank 146 by a pair of brackets 155—155. A scraper 160 scrapes the cathode tape 144 to remove metal plated on that tape by the electropolishing process.

*Operation of the embodiment shown in Figs. 5 to 8*

The tape 110 is advanced continuously through the baths 112, 114, 118, 120, 122 and 124. The bath 112 cleans grease and other foreign matter from the tape, and the water rinsing bath 114 rinses the alkali from the tape. The cathode tape 144 is advanced through the bath 118 along the tape 110 at the same rate of speed as that of the tape 110. During the initial portion of the passage of the tape 110 through the bath 118, the resistance between the tapes 110 and 144 is sufficiently high to prevent rapid passivation of the front face of the tape 110, but

is sufficiently low to cause all larger projections on the front face of the tape 110 to be electrolytically dissolved rapidly.

The current density on the front face of the tape 110 increases as it moves from the entrance end of the bath 118 toward the exit end thereof because of the continuous shortening of the path between the two tapes. As the current density increases, the portion of the electrolyte immediately adjacent to the front face of the tape 110 is broken down to provide oxygen, which reacts with the copper coming from the tape to form oxides on the front face of the tape 110. This face of the tape below the oxides is polished highly by the time the oxides build up to a passivating condition. Slightly before the tape 110 leaves the bath 118, this passivating condition is reached which reduces current flow to a small amount. Thus, the passivation acts as a control to stop substantially further dissolution of copper from the tape 110.

After passivation, the front of the tape 110 has an oxide layer having a lustrous, straw color thereon. This oxide layer is removed from the conductor by the alkaline neutralizing bath 122, which dissolves it and leaves a smooth, golden surface on the front face of the tape.

The movement of the tape 110 through the electro-polishing bath 118 is sufficiently slow to prevent agitation around the front face of the portion of the tape in the bath 118. As a result, the breakdown of electrolyte produced along the front face of the tape by the electrolytic action is such that there is sufficient oxygen available at the front face of the tape to form the passivating layer of copper oxides, which limits polishing of this surface when it has become smooth.

In one successful example, the tape 110 was 1 1/8 inches in width, each portion of the front face of a tape, except the serrated edge portions, was subjected to electrolytic polishing in an electropolishing bath for a period of from 10 to 15 seconds, and the bath was about four feet long. The cathode tape 144 also was 1 1/8 inches in width, the spacing between the tapes 110 and 144 varied from 1 1/2 inches at the entrance end of the bath to 3/4 inch at the exit end thereof, and the potential difference between the tapes was 18 volts. The current density on the face of the tape being polished increased gradually and uniformly from the entrance end of the bath to the exit end thereof, near which the anode current density was over 3,000 amperes per square foot. The average current density on that face of the tape was 1,600 amperes per square foot. The electropolishing bath employed was identical with that used in the previous embodiment of the invention, and it was maintained at about 85° F.

Certain features of the above-described methods and apparatus are disclosed and claimed in my copending application Serial No. 175,125, filed July 21, 1950, for "Methods of and Apparatus for Electropolishing Metallic Articles," and in copending application Serial No. 175,189, filed July 21, 1950, by A. N. Gray for "Methods of and Apparatus for Electropolishing Metallic Articles."

Copper articles of a nonfilamentary type may be held stationary in the several baths described hereinabove, and stationary cathodes may be used to successfully polish the articles. Such articles may also be advanced continuously through the baths with or without moving electrodes. Such stationary articles may be polished satisfactorily without continuously increasing the current density thereon in the electropolishing bath, while keeping an average anode polishing current density of the order of 3,000 amperes per square foot.

The above-described methods rapidly form lustrous, highly polished surfaces on copper articles originally having minute projections on the surfaces thereof, and the polished surfaces have no pits therein. While the conductor 10 and the tape 110 described hereinabove were made of copper, composite metallic articles having a core

composed of one metal, such as, for example, steel and a covering of copper may be successfully electropolished by means of the above-described methods. These methods also may be used in conjunction with suitable electrolytes to successfully electropolish other metals, such as steel, brass, zinc, nickel, stainless steel, etc.

In the use of terms, such as "filament" and "filamentary article," and the like, in the specification and claims, it is intended to include rods, wires, tapes, bands, and the like.

What is claimed is:

1. The method of electropolishing copper articles, which comprises making a copper article an anode in an electrolytic cell including an aqueous bath consisting essentially of from about 18% to about 30% copper nitrate, from about 6% to about 2% sulphuric acid and the balance water, and impressing a D. C. potential upon the cell of sufficient magnitude to maintain an average anode current density of at least 3,000 amperes per square foot and to simultaneously release sufficient oxygen from the bath around the article to passivate the surface thereof with copper oxides and highly polish the surface of the article beneath the oxides.

2. The method of electropolishing copper filaments, which comprises advancing a copper filament as an anode 25 through an electrolytic cell including an aqueous bath consisting essentially of from about 18% to about 30% copper nitrate, from about 6% to about 2% sulphuric acid and the balance water without agitating the bath materially, impressing a D. C. potential upon the cell of 30 sufficient magnitude to create an average current density on the filament of at least 3,000 amperes per square foot, maintaining a current density on the portion of the filament in that portion of the bath near the entrance end thereof sufficiently low not to cause passivation of the 35 surface of that portion of the filament but sufficiently high to remove projections from the surface of the filament, and maintaining a current density on the filament between said portion and the exit end of the bath sufficiently high to release sufficient oxygen from the bath around the 40 filament to passivate the surface thereof with copper oxides.

3. The method of electropolishing copper articles, which comprises electrolyzing a copper article to be polished as an anode in an electrolyte consisting of copper 45 nitrate about 19% by weight, sulphuric acid about 4.5% by weight and the balance water, maintaining the electrolyte at a temperature of from about 75° F. to about 90° F., impressing a D. C. potential upon the cell to create an anode current density adequate to polish the article, and continuing the electrolysis until the surface of the 50 article is passivated.

4. The method of electropolishing copper articles, which comprises immersing a copper article in an electrolytic cell containing an aqueous electrolyte consisting essentially of from about 18% to about 30% copper nitrate, from about 6% to about 2% sulphuric acid and the balance water, impressing a D. C. potential upon the cell of sufficient magnitude to create an anode current density on the article adequate to polish the article, and maintaining such potential until eventually sufficient oxygen is released from the electrolyte to passivate the surface of the article by forming an oxide coating thereon.

5. The method of electropolishing copper filaments, which comprises advancing a copper filament as an anode 65 through an electrolytic cell containing an aqueous electrolyte consisting essentially of from about 18% to about 30% copper nitrate, from about 6% to about 2% sulphuric acid and the balance water, impressing a D. C. potential upon the cell of sufficient magnitude to create an anode current density on the filament adequate to polish the filament, and gradually increasing the current density until eventually sufficient oxygen is released from the electrolyte to passivate the surface of the filament by forming an oxide coating thereon.

6. The method of electropolishing copper filaments,

which comprises advancing a copper filament as an anode through an electrolytic cell containing an aqueous electrolyte consisting essentially of from about 18% to about 30% copper nitrate, from about 6% to about 2% sulfuric acid and the balance water, maintaining the temperature of the electrolyte at from about 75° F. to about 90° F., impressing a D.C. potential upon the cell of sufficient magnitude to create an anode current density on the filament adequate to polish the filament, and gradually increasing the current density sufficiently to release oxygen from the electrolyte and eventually to cause the surface of the filament to become passivated rapidly by forming an oxide coating thereon.

|           |                 |                |
|-----------|-----------------|----------------|
| 2,023,998 | Fustier         | Dec. 10, 1935  |
| 2,330,170 | Manuel          | Sept. 21, 1943 |
| 2,378,002 | Drummond et al. | June 12, 1945  |
| 2,542,779 | Neill           | Feb. 20, 1951  |

## OTHER REFERENCES

"Hackh's Chemical Dictionary," second edition (1937), pages 162, 163, definition of "buffer."

"Transactions of The American Electrochemical Society," vol. 23 (1913), page 250 of article by Bennett.

"Proceedings of The American Electroplaters Society," June 1946, page 51 of article by Faust.

"Metal Industry," New York, June 8, 1945, pages 357 and 358 of article by Crout.

References Cited in the file of this patent 15

## UNITED STATES PATENTS

1,773,160. Anderson et al. Aug. 19, 1930